# EUROPEAN PATENT SPECIFICATION

(11) **EP 2 646 602 B1**
(45) Date of publication and mention of the grant of the patent: **27.04.2016**
(21) Application number: 11731520.0
(22) Date of filing: 10.06.2011
(51) Int. Cl.: C25D 5/02, C25D 7/00, C25D 7/12, G21K 1/06, H01L 21/768

(54) **METHOD OF MANUFACTURING AN X-RAY DIFFRACTION GRATING MICROSTRUCTURE FOR IMAGING APPARATUS**
VERFAHREN ZUR HERSTELLUNG EINER MIKROSTRUKTUR EINES RÖNTGEN-DURCHSTRAHLUNGSGITTERS FÜR EIN BILDAUFNAHMEGERÄT
MÉTHODE DE MANUFACTURE D'UNE MICROSTRUCTURE EN RÉSEAU DE DIFFRACTION DE RAYONS X POUR UN APPAREIL D'IMAGERIE

(30) Priority: 29.11.2010 JP 2010265093
(43) Date of publication of application: 09.10.2013
(73) Proprietor: Canon Kabushiki Kaisha, Tokyo 146-8501 (JP)
(72) Inventor: WANG, Shinan, Tokyo 146-8501 (JP); NAKAMURA, Takashi, Tokyo 146-8501 (JP); TESHIMA, Takayuki, Tokyo 146-8501 (JP); SETOMOTO, Yutaka, Tokyo 146-8501 (JP); WATANABE, Shinichiro, Tokyo 146-8501 (JP)
(74) Representative: TBK
(86) International application number: PCT/JP2011/063989
(87) International publication number: WO 2012/073545

(56) References cited:
- WO-A2-2009/113726
- DE-A1-102006 037 281
- JP-A- 2006 259 264
- JP-A- 2008 197 593
- JP-A- 2010 185 728
- US-A1- 2003 134 510

## Description

### Technical Field

The present invention relates to a microstructure manufacturing method for manufacturing a microstructure by electrolytic plating, an X-ray absorption grating obtainable by this method, and an imaging apparatus using the X-ray absorption grating.

### Background Art

A micro fine structure having periodic structure, especially a high aspect ratio structure is needed in a large number of fields. For example, the X-ray absorption characteristic of a microstructure composed of gold is utilized in a nondestructive test of an object as an industrial application, and also utilized in, for example, radiography as a medical application. A microstructure in these applications forms a contrast image by utilizing an absorption difference in X-ray transmission depending on constituent elements and a density variation in an object or a biological object, and is called the X-ray absorption contrast method.

Further, the phase contrast method using a phase difference of X-ray has been researched actively since even light elements can be imaged by this method, and for example, the propagation method and the Talbot interference method has been becoming feasible in principle. Generally, the method using Talbot interference is carried out with use of an absorption grating comprised of gold having a periodic structure and large absorption of X-ray. Since it is difficult to directly manufacture a golden microstructure having a high aspect ratio ("aspect ratio" is defined as a ratio of a height or depth h and a width w of a structure (h/w)), the method of filling a mold with gold by plating is preferable as a method for manufacturing a golden absorption grating constituted by a periodic structure.

PTL 1 discusses a structure of an X-ray optical transmission grating for the above-described phase contrast method. Further, with the aim of solving the problem of a significant reduction in fabrication precision according to an increase in the aspect ratio of a structure, PTL 1 discusses a combination of partial gratings which functions as one grating.

However, PTL 1 does not discuss a method for manufacturing a microstructure having a high aspect ratio.

### Citation List

### Patent Literature

PTL 1 Japanese Patent Laid-Open No. 2007-203066

### Summary of Invention

The present invention is directed to a microstructure manufacturing method enabling easy manufacturing of a metal microstructure having a high aspect ratio with a high degree of precision, an X-ray absorption grating obtainable by the microstructure manufacturing method, and an imaging apparatus using the X-ray absorption grating.

According to an aspect of the present invention, there is provided a microstructure manufacturing method as defined in claim 1. According to another aspect of the present invention, there is provided an X-ray absorption grating as defined in claim 9 and an imaging apparatus as defined in claim 14.

Further features and aspects of the present invention will become apparent from the following detailed description of exemplary embodiments with reference to the attached drawings.

### Brief Description of Drawings

The accompanying drawings, which are incorporated in and constitute a part of the specification, illustrate exemplary embodiments, features, and aspects of the invention and, together with the description, serve to explain the principles of the invention.
**[****Figs. 1A-1G]** Figs. 1A to 1G illustrate a microstructure manufacturing method according to a first exemplary embodiment of the present invention.
**[****Figs. 2A-2H]** Figs. 2A to 2H illustrate a microstructure manufacturing method according to a second exemplary embodiment of the present invention.
**[****Figs. 3A-3J]** Figs. 3A to 3J illustrate a microstructure manufacturing method according to a third exemplary embodiment of the present invention.
**[****Fig. 4A]** Fig. 4A illustrates a typical substrate (wafer) according to exemplary embodiment of the present invention.
**[****Fig. 4B]** Fig. 4B illustrates a pattern on the substrate according to the exemplary embodiment of the present invention.
**[****Figs. 5A-5G]** Figs. 5A to 5G illustrate a fourth exemplary embodiment of the microstructure manufacturing method of the present invention.
**[****Fig. 6]** Fig. 6 illustrates a structure of an imaging apparatus according to the exemplary embodiments of the present invention.

### Description of Embodiments

Various exemplary embodiments, features, and aspects of the invention will be described in detail below with reference to the drawings.

Fig. 1 illustrates a first exemplary embodiment of the microstructure manufacturing method according to the present invention. This manufacturing method is a method including forming a microstructure on one surface of an Si substrate, and forming a metal microstructure by applying electrolytic plating to the inside of the Si microstructure while using the Si microstructure as a mold.

First, a first insulating film is formed on the front surface and the back surface of the Si substrate (first process). As illustrated in Fig. 1A, the first insulating film 20 is formed on a front surface 1 and a back surface 2 of an Si substrate 10. The size and thickness of the Si substrate 10 can be determined according to a desired microstructure. Further, the resistivity of the Si substrate 10 is 10 Ωcm or less, preferably or optimally 0.1 Ωcm or less.

The material of the first insulating film 20 is an insulating material having resistivity sufficiently high relative to the Si substrate 10. Preferably, the resistivity of the first insulating film 20 is equal to or more than ten times the resistivity of the Si substrate 10. Preferably, the first insulating film 20 can offer sufficient selectivity ratio, and can be used as a mask material in the later processing of an Si microstructure. Preferably, the material of the first insulating film 20 is, for example, SiO₂ or an Si nitride film. Preferably, the thickness of the first insulating film 20 is 0.1 µm or more, and 5 µm or less. Examples of SiO₂ film formation methods include the thermal oxidation method and the chemical vapor deposition (CVD) method. Examples of Si nitride film formation methods include the chemical vapor deposition (CVD) method. Preferably, the first insulating film 20 is formed on both of the front surface and the back surface of the substrate.

Next, the Si surface of the Si substrate is exposed by removing a part of the first insulating film on the front surface of the Si substrate (second process). As illustrated in Fig. 1B, a mask pattern 21 is formed by removing a part of the first insulating film 20, and at the same time, an Si surface 11 portion is formed by partially exposing the front surface of the Si substrate 10. The partial removal of the first insulating film 20 will be described based on the case that the material of the first insulating film 20 is SiO₂ by way of example. For example, after a metal film (for example, Cr) is formed on the first insulating film 20, a photoresist (for example, AZ1500: manufactured by AZ Electronic Materials Company) is applied thereon. Then, the photoresist is exposed to light for the formation of a pattern. The shape and size of the pattern is determined based on a desired metal microstructure. For example, the pattern may be constituted by a periodic structure of a square pattern, the period of which is approximately 1 µm to 100 µm and a length of one side of which is 0.5 µm to 80 µm. Then, the photoresist pattern is transferred onto the metal film by etching. The metal film etching method may be embodied by a wet etching method with use of a solution or a dry etching method such as ion sputtering and reactive gaseous plasma etching. After that, the first insulating film 20 is etched using the metal film with the pattern transferred thereon as a mask. For example, preferably, the etching of the first insulating film 20 is carried out by a dry etching method. If the first insulating film 20 is made of SiO₂, preferably, the etching is carried out by the dry etching method with use of CHF₃ plasma.

Next, the Si recessed portion is formed by etching the Si substrate from the exposed Si surface using the first insulating film on the front surface of the Si substrate as a mask (third process). As illustrated in Fig. 1C, an Si recessed portion 12 is formed by processing the Si substrate 10 from the Si surface 11 portion exposed by the partial removal of the first insulating film 20 using the pattern 21 on the first insulating film formed by the previous processing as a mask. Fig. 1C illustrates each of a sidewall 13 and a bottom 14 of the Si recessed portion 12. The method of processing the Si substrate 10 may be embodied by a wet etching method with use of a solution or a dry etching method such as ion sputtering and reactive gaseous plasma etching. Especially, out of the reactive gaseous plasma dry etching methods, reactive ion etching (RIE) is suitable for manufacturing a high aspect ratio structure. Further especially, out of RIE, Bosch process RIE, which alternately repeats etching by SF₆ gas and sidewall protective film deposition by C₄F₈ gas, is further suitable for manufacturing a high aspect ratio structure. Use of Bosch process RIE enables manufacturing of a structure having an aspect ratio of approximately 100. Desirably, if the Bosch process RIE is carried out, the sidewall protective film is removed after the RIE. The removal of the sidewall protective film can be carried out by, for example, cleaning with use of a hydro fluoro ether (HFE) solution.

Next, a second insulating film is formed on the sidewall and the bottom of the Si recessed portion (fourth process). As illustrated in Fig. 1D, a second insulating film 30 is formed on the sidewall 13 and the bottom 14 of the Si recessed portion 12 formed by the previous processing. The material of the second insulating film 30 may be the same as or different from the material of the above-described first insulating film 20. For example, both the material of the first insulating film 20 and the material of the second insulating film 30 are SiO₂. Alternatively, the material of the first insulating film 20 is SiO₂, and the material of the second insulating film 30 is a Silicon nitride film. Alternatively, the material of the first insulating film 20 is an Si nitride film, and the material of the second insulating film 30 is SiO₂. The thickness of the second insulating film 30 is within the range of 5 nm to 5000 nm, preferably 10 nm to 1000 nm, most preferably 20 nm to 200nm. The thickness of the second insulating film 30 does not necessarily have to be even throughout the Si recessed portion 12 and the region of the sidewall 13, and only have to be 10 nm or more at the thinnest portion. More preferably, the second insulating film 30 has the thinnest thickness at a portion denoted by reference numeral 34 (the bottom 14 of the Si recessed portion 12). The second insulating film 30 may be formed on a portion other than the sidewall 13 and the bottom 14 (for example, on the top portion 21 of the substrate or the back surface of the substrate).

Next, the Si exposed surface is formed by at least partially removing the second insulating film formed on the bottom of the above-described Si recessed portion (fifth process). As illustrated in Fig. 1E, an Si exposed surface 15 is formed by at least partially removing the second insulating film 34 formed on the bottom 14 of the Si recessed portion 12. Preferably, the partial removal of the second insulating film 34 is carried out by a highly anisotropic dry etching method. For example, the removal of the second insulating film 34 is carried out by the ion sputtering method or the reactive gaseous plasma etching method. In such a method, since the second insulating film 34 at the bottom is preferentially removed due to the anisotropy of the etching, the second insulating film 34 can remain at the sidewall at least thinly, preventing the Si surface from being exposed at the sidewall. Further, if the insulating film on the top surface of the substrate is made to be sufficiently thicker than the second insulating film 34 on the bottom, this enables the Si surface on the top surface of the substrate to be prevented from being exposed when the second insulating film 34 is removed. If the second insulating film 34 is made of SiO₂, the removal thereof is preferably carried out by the dry etching method with use of CHF₃ plasma. The Si exposed surface 15 illustrated in Fig. 1E corresponds to the bottom 14 of the Si recessed portion. As illustrated in Fig. 1G, it is also convenient for carrying out the present exemplary embodiment to further expose a sidewall 17 of the Si recessed portion adjacent to the bottom 14 by further processing the bottom 14 after the bottom 14 is exposed, if desired. Execution of the above-described processes results in the formation of an Si mold 40 for plating.

Next, a metal microstructure is formed by filling the Si recessed portion with a metal from the above-described Si exposed surface by electrolytic plating (sixth process). As illustrated in Fig. 1F, a metal microstructure 50 is formed by electrolytic plating the inside 12 of the Si structure with a metal from the Si exposed surface 15 while using the Si mold 40 as a mold. In the Si mold 40, an exposed surface is only the surface of the bottom of the Si recessed portion which constitutes the Si exposed surface 15, and the other portions including the back surface of the substrate are all covered with the insulating film. Therefore, in the electrolytic plating, the metal can be deposited only from the Si exposed surface 15. As a result, a fine metal microstructure can be manufactured within the recessed portion 12 of the Si mold 40. The metal may be embodied by any metal enabling a formation of a microstructure by electrolytic plating, for example, preferably Au and Ni. An electrode pad for the mold side for the electrolytic plating may be formed at, for example, the periphery of the front surface of the Si substrate 10 or the back surface of the Si substrate 10. In this case, the electro pad formation method may be embodied by, for example, the method of removing the first insulating film 20 and the second insulating film 30 at an appropriate position at the periphery of the Si substrate 10 or the back surface of the Si substrate 10 to expose the surface of the Si substrate after the completion of the formation of the Si mold 40 till the process of Fig. 1E. Alternatively, for the electro pad, an Si recessed portion having an area suitable for an electro pad may be formed at an appropriate position at the periphery of the front surface of the Si substrate 10, at the same time of the formation of the Si recessed portion 12 as illustrated from Figs. 1A to 1E.

The above-described processes of the manufacturing method may be carried out with support from the well known Micro Electro Mechanical System (MEMS) technology. Further, the present exemplary embodiment does not require additional formation of a seed electrode which would be required in an ordinary electrolytic plating process, and reduces the number of manufacturing processes. Especially, the present exemplary embodiment does not require a difficult technology for selectively forming a seed electrode at the bottom of a high aspect ratio structure, and realizes easy manufacturing.

According to the present exemplary embodiment, it is possible to manufacture a metal micro grating structure having an aspect ratio of 0.1 to 150, preferably 5 to 100, with a high degree of submicron precision.

Figs. 2A to 2H illustrate a second exemplary embodiment according to the microstructure manufacturing method of the present invention. Figs. 2A to 2H illustrate the second exemplary embodiment of the present invention. The following description will disclose a microstructure manufacturing method including forming microstructures on the both surfaces of an Si substrate, and forming metal microstructures in the microstructures by electrolytic plating while using the microstructures as molds.

First, the first insulating film is formed on the front surface 1 and the back surface 2 of the Si substrate (first process). Next, the Si surface of the Si substrate is exposed by removing a part of the first insulating film on the front surface of the Si substrate, and then the Si recessed portion is formed on the front surface of the Si substrate by etching the Si substrate from the exposed Si surface while using the first insulating film on the front surface of the Si substrate as a mask (second process).

More specifically, as illustrated in Figs. 2A to 2C, the Si microstructure is formed on the front surface of the Si substrate 10. The formation method therefor can be carried out in a similar manner to the method of the first exemplary embodiment as illustrated in Figs. 1A and 1C.

Next, the Si surface of the Si substrate is exposed by removing a part of the first insulating film on the back surface of the Si substrate, and then the Si recessed portion is formed on the back surface of the Si substrate by etching the Si substrate from the exposed Si surface while using the first insulating film on the back surface of the Si substrate as a mask (third process).

As illustrated in Fig. 2D, the Si recessed portion corresponding to the Si recessed portion formed on the front surface of the Si substrate 10 is formed on the back surface of the Si substrate 10 in a substantially mirror-symmetrical manner by applying processing from the back surface. In other words, the Si recessed portions are formed on the front surface and the back surface of the Si substrate so as to establish a mirror-symmetrical relationship therebetween. Preferably, the Si microstructure on the back surface is substantially mirror-symmetrical to the Si microstructure on the front surface as viewed in a planar figure. When a photoresist pattern is formed on the back surface, the position thereof is aligned to the Si recessed portion on the front surface of the Si substrate with use of a position alignment mark formed in advance on the front surface of the Si substrate, in order to precisely set the positional relationship between the Si recessed portions on the front surface and the back surface. On the other hand, the Si recessed portions on the front surface and the back surface do not have to have a same depth. Preferably, an intermediate layer 16, which is defined between the Si recessed portions on the front surface and the back surface, is thin. For example, the thickness of the intermediate layer 16 may be 500 µm or less, more preferably 50 µm or less. Such a dimension can be realized by determining the thickness of the Si substrate 10 in consideration of the thickness of the intermediate layer 16.

Next, the second insulating films are formed on the sidewalls and the bottoms of the Si recessed portions on the front surface and the back surface of the Si substrate (fourth process). As illustrated in Fig. 2E, the second insulating films 30 are formed on the sidewalls 13 and the bottoms 14 of the Si recessed portions 12 formed by the previous processing. At this time, the second insulating films 30 may be formed on the Si recessed portions on the front surface and the back surface either concurrently or separately. Further, the materials of the second insulating films 30 formed on the Si recessed portions on the front surface and the back surface may be either substantially similar to each other or different from each other. The details of the second insulating film 30 such as the formation method thereof and the dimension of the thickness thereof may be similar to the second insulating film 30 in the first exemplary embodiment as illustrated in Fig. 1D.

Next, the Si exposed surfaces are formed by at least partially removing the second insulating films formed on the bottoms of the Si recessed portions on the front surface and the back surface of the Si substrate (fifth process). As illustrated in Fig. 2F, the Si exposed surface 15 is formed by at least partially removing the second insulating film 34 formed on the bottom 14 of the Si recessed portion 12. This process is performed for each of the Si recessed portions on the front surface and the back surface. The method of partially removing the second insulating film 34 may be similar to the method of removing the second insulating film 34 in the first exemplary embodiment as illustrated in Fig. 1E. Execution of the above-described processes illustrated in Figs. 2A to 2F results in the formation of the Si molds 40 on the both surfaces of the substrate, which are constituted by the Si recessed portions for plating of Si microstructures.

Next, metal microstructures are formed by filling the Si recessed portions with metals from the Si exposed surfaces on the front surface and the back surface of the Si substrate by electrolytic plating (sixth process). As illustrated in Figs. 2G and 2H, the metal microstructures 50 are formed on the both surfaces of the Si substrate by electrolytic plating the insides 12 of the Si recessed portions with metals from the Si exposed surfaces 15 while using the Si molds 40 as molds. The metal electrolytic plating method may be similar to the metal electrolytic plating method in the first exemplary embodiment as illustrated in Fig. 1F.

According to the present exemplary embodiment, it is possible to manufacture a metal structure having a high aspect ratio on each of the both surfaces of an Si substrate. This is effective in many applications. For example, in the case of an X-ray absorption grating, the present exemplary embodiment can provide, as a total effect, an X-ray absorption effect substantially corresponding to a simple sum of the absorption effects of the metal microstructures on the front surface and the back surface. In other words, formation of metal microstructures on the both surfaces of an Si substrate enables the metal microstructure to have an aspect ratio corresponding to the sum of the aspect ratios of the metal microstructures on the front surface and the back surface. For example, if metal microstructures on the front surface and the back surface are substantially the same, the collective metal microstructure has an overall aspect ratio approximately twice compared to a metal microstructure having the microstructure formation only on one surface.

Further, the plating is carried out simultaneously from the both surfaces of the mold, whereby the time required for plating can be significantly reduced compared to plating performed for one surface at a time. Another effect of the present exemplary embodiment is improvement of the processing accuracy. In this method, the processing accuracy of a metal microstructure is generally determined based on an Si microstructure. Since the processing of an Si microstructure is substantially similar to the processing of an Si microstructure only on one surface, the processing accuracy is also substantially similar to the processing accuracy of an Si microstructure only on one surface. Further, even if a metal structure has an aspect ratio enabling the one-side formation, it is possible to reduce the processing difficulty and improve the processing accuracy by employing the formation on the both surfaces. An increase in the processing difficulty and a reduction in the processing accuracy first occur when a Si microstructure mold with a high aspect ratio is formed, and are more noticeable as an aspect ratio becomes higher. Especially, a structure having an aspect ratio of 50 or more often raises problems such as disarray and tilt of the Si microstructure, thereby resulting in strict processing conditions and a reduction in the processing rate.

In plating of an Si microstructure mold with a metal, a higher aspect ratio leads to difficulty in the entry of a plating solution into the bottom of the Si recessed portion, and bad circulation of the plating solution within the recessed portion. As a result, the plating should be carried out at a reduced plating rate, thereby deteriorating the productivity. Further, a higher aspect ratio may lead to uneven application of plating in the Si recessed portion and generation of voids in the metal structure. The present exemplary embodiment is highly effective for solving the above-described problems. According to the present exemplary embodiment, it is possible to comparatively easily manufacture a metal micro grating structure having a high aspect ratio of approximately 200 with a high degree of submicron precision.

Figs. 3A to 3B illustrates a third exemplary embodiment according to the microstructure manufacturing method of the present invention. The third exemplary embodiment is a method including forming an Si mold by penetratingly connecting the microstructures formed on the both surfaces of the Si substrate, and forming a metal microstructure by electrolytically plating the inside of the Si mold.

More specifically, by etching of the Si substrate from the exposed Si surfaces while using the first insulation films on the front surface and the back surface of the Si substrate as masks, the Si recessed portions on the front surface and the back surface of the Si substrate can be formed either in a manner that the respective Si recessed portions penetrate or in a manner that the respective Si recessed portions do not penetrate. The present exemplary embodiment employs the method that the Si recessed portions are formed in a manner that the respective Si recessed portions penetrate. In this method, a part of the bottom and/or a part of the sidewall of the Si recessed portion can serve as the Si exposed surface.

First, as illustrated in Figs. 3A to 3G, the Si substrate 10 is processed so as to have the Si recessed portion which serves as the Si mold 40. The processes illustrated in Figs. 3A to 3F may be similar to the processes in the second exemplary embodiment as illustrated in Figs. 2A to 2F. In the present exemplary embodiment, the Si substrate 10 in the state illustrated in the Fig. 3F is processed so that the intermediate layer 16 defined between the Si recessed portions on the front and back surfaces is at least partially removed to penetratingly connect the Si recessed portions on the front and back surfaces, as illustrated in Fig. 3G. This processing results in the formation of the exposed surface 17 on the sidewall of the Si recessed portion. The removal of the Si intermediate layer 16 here may be performed in a similar manner to the removal in the first exemplary embodiment as illustrated in Fig. 1C. Execution of the processes illustrated in Figs. 3A to 3G results in the formation of the Si mold 40 including the penetrating Si recessed portion.

Next, as illustrated in Figs. 3H to 3J, the metal microstructure 50 is manufactured by electrolytically plating the inside 12 of the Si structure with a metal from the Si exposed surface 17 while using the Si mold 40 including the penetrating Si recessed portion. The metal electrolytic plating method may be substantially similar to the metal electrolytic plating method in the first and second exemplary embodiments, except for a difference which will be now described. First, unlike the first and second exemplary embodiments, the present exemplary embodiment includes the penetrating Si microstructure constituted by the Si recessed portion, and the Si exposed surface 17 formed mainly on the sidewall of the recessed portion of the Si microstructure. Therefore, during electrolytic plating of a metal, the metal is deposited only on the Si exposed surface 17 in initial stage, as illustrated in Fig. 3H. After a while, the passage of the plating solution in the Si microstructure is closed by the deposited metal 50, as illustrated in Fig. 3I. Then, the metal plating is continued to form the desired metal microstructure 50, as illustrated in Fig. 3J.

According to the present exemplary embodiment, it is possible to manufacture a metal microstructure having a high aspect ratio in the penetrated Si mold. In this case, the following effects can be provided in addition to the effects of the second exemplary embodiment. The penetration of the Si microstructure results in the improvement of the circulation of the plating solution within the Si microstructure constituted by the Si recessed portion, compared to the plating without penetration of the Si microstructure. Therefore, it is possible to further facilitate the plating within the Si microstructure. Especially, it is possible to speed up the formation of a plating core in an early stage of plating. This state is maintained until the passage in the Si microstructure is closed by the metal 50 (Fig. 3I). Further, since the metal microstructure manufactured by the present exemplary embodiment has an integrated structure, it can provide more excellent element characteristics.

In a first example, as illustrated in Figs. 1A to 1G, an Si microstructure was formed on one surface of an Si substrate, and an Au microstructure was formed by electrolytically plating the inside of the Si microstructure while using the Si microstructure as a mold. First, as illustrated in Fig. 1A, the first insulating film 20 was formed on the Si substrate 10. The Si substrate had a diameter of 100 mmϕ, a thickness of 400 µm, and a resistivity of 0.02 Ωcm. The material of the first insulating film 20 was SiO₂. The wet thermal oxidation method was employed as the SiO₂ film formation method. The SiO₂ film with a thickness of approximately 1.2 µm was formed on each of the front surface and the back surface of the Si substrate 10 by thermal oxidation performed at 1050 °C for four hours. The resistivity of the SiO₂ film was 1000 Ωcm or more.

Next, as illustrated in Fig. 1B, the mask pattern 21 was formed by removing a part of the above-described first insulating film SiO₂, and at the same time, the surface of the Si substrate 10 was partially exposed to form the Si surface 11 portion. More specifically, first, a Cr film with a thickness of 100 nm was deposited on the SiO₂ as a metal film by the vacuum deposition method. Then, AZ1500 with a thickness of approximately 3 µm was applied on the Cr film as a photoresist. After that, the photoresist was exposed to light to form a desired pattern. As illustrated in Fig. 4A, the pattern 60 was disposed at approximately the center of the front surface of the substrate 10, and the diameter thereof was approximately 50 mmϕ. As illustrated in Fig. 4B, the pattern was a periodic structure, and was an array of squares 4 µm on a side (W=4µm) at 8 µm intervals (p = 8 µm).

Next, the photoresist pattern was transformed onto the Cr by etching the Cr with use of a commercially available Cr etching solution. Then, the SiO₂ was etched by the CHF₃ plasma dry etching method with use of the Cr pattern as a mask to expose the Si surface portion 11. After that, the Cr film was all removed with use of the above-described etching solution, as a result of which the Si substrate 10 was covered with the SiO₂ pattern 21 while the surface portion 11 of the Si substrate 10 was exposed as illustrated in Fig. 4B. At this time, as illustrated in Fig. 4A, a square pattern approximately 1 mm on a side was formed at the periphery of the substrate 10 concurrently so that the electric pad 70 was formed.

Next, as illustrated in Fig. 1C, the Si substrate 10 was processed, with use of the SiO₂ pattern 21 as a mask, to form an array structure constituted by Si square poles. The method for processing the Si substrate 10 was the Bosch process RIE method, which alternately repeats etching with use of SF₆ gas and sidewall protective film deposition with use of C₄F₈ gas. After the execution of Bosch process RIE, the substrate was cleaned with a hydro fluoro ether (HFE) solution and a mixed solution of sulfuric acid and hydrogen peroxide for removing the sidewall protective film.

A cross-sectional observation of the Si structure with a scanning electron microscope (SEM) revealed that the height of the Si square pole was approximately 240 µm. Further, a research of the cross-sectional shape of the Si square pole after cutting the Si square pole with focused ion beam (FIB) revealed that the Si square pole was nearly square in cross-section. Although the Si square was approximately 4 µm on a side near the surface of the recessed portion, the Si square was approximately 3.6 µm on a side near the bottom of the recessed portion. Therefore, the obtained Si square pole had an aspect ratio of approximately 60. Further, an SEM cross-sectional observation revealed that the SiO₂ film 21 with a thickness of 0.2 µm or more remained on the Si square pole.

Next, as illustrated in Fig. 1D, the second insulating film 30 was formed on the sidewall 13 and the bottom 14 of the Si recessed portion 12 formed by the previous processing. In this example, SiO₂ was selected for the second insulating film 30, too. The film thickness of the second insulating film 30 was approximately 100 nm. The method for forming the second insulating film 30 was thermal oxidation as illustrated in Fig. 1A. The preferable feature of thermal oxidation is that it enables the formation of a highly dense SiO₂ film with a comparatively even thickness. This processing causes thermal oxidation to progress even at the portions other than the sidewall 13 and the bottom 14, i.e. , the substrate top 21 covered with the SiO₂ film or the back surface of the substrate, and provides an increase in the film thickness of the SiO₂ film. This is advantageous to the later processes.

Next, as illustrated in Fig. 1E, the SiO₂ film 34 formed on the bottom 14 of the Si recessed portion 12 was removed to form the Si exposed surface 15. The partial removal of the SiO₂ film 34 was carried out by the dry etching method with use of CHF₃ plasma. This etching has high anisotropy and progresses nearly vertically relative to a substrate. Therefore, while the SiO₂ film 34 at the bottom was completely removed, the SiO₂ film on the sidewall remained so that Si of the sidewall was prevented from being exposed. On the other hand, the thickness of the SiO₂ film 21 on the substrate top was increased compared to the thickness of the film at the time of Fig. 1C which was 0.2 µm or more due to the thermal oxidation illustrated in Fig. 1D, as a result of which the SiO₂ film 21 remained even though the SiO₂ film 34 was completely removed so that the Si surface was prevented from being exposed at this portion. The above-described processes led to the formation of the Si mold 40 for plating, which had an Si exposed surface only at the bottom of the recessed portion while the other portions were covered with the SiO₂ film of a high resistivity.

Next, as illustrated in Fig. 1F, the Au microstructure 50 was formed by electrolytically plating the inside 12 of the Si structure with Au from the Si exposed surface 15 while using the portion 40 as a mold. Microfab Au1101 (manufacturer: Electroplating Engineers of Japan Ltd.) was used as an Au plating solution. At the time of the plating, the temperature of the plating solution was maintained at 60 °C, and the current density was set to 0.2 A/dm². The plating solution was stirred to ensure even application of plating. The Si exposed surface 70 illustrated in Fig. 4A was utilized as an electrode pad for the mold side for the electrolytic plating.

The Si mold 40 had an exposed surface at the bottom of the Si recessed portion indicated as the Si exposed surface 15, and the other portions of the Si mold 40 were entirely covered with the SiO₂ film which was an insulating film. Therefore, at the time of the electrolytic plating of Au, Au was deposited only on the Si exposure surface 15 to form a dense Au microstructure within the recessed portion 12 of the Si mold 40.

The height of the Au microstructure 50 was controlled by the plating time so as to become approximately 200 µm. In other words, the aspect ratio of the obtained Au microstructure was approximately 50. A cross-sectional observation with, for example, a SEM revealed that the Au microstructure was dense and had no void. Further, an evaluation with an X-ray microscope confirmed that a grating image with clear contrast could be obtained, and the Au microstructure could absorb X-ray.

As indicated by the present example, element technologies required for the first exemplary embodiment are all derived from the well-known MEMS technology, and therefore can be readily carried out. Especially, the first exemplary embodiment employs the idea of using a highly processible Si substrate as a mold and enabling Au to be deposited only from the conductive bottom of the recessed portion of the mold by covering the surface of the mold with an insulating SiO₂ film, whereby it is possible to manufacture a metal micro grating structure having a high aspect ratio with a reduced number of manufacturing processes with a high degree of submicron precision. Further, the first exemplary embodiment uses an SiO₂ film which can prevent unnecessary Au deposition to, for example, the sidewall of the mold, and improve the selectivity of a plating solution for the Au plating.

In a second example, as illustrated in Figs. 2A to 2H, Si microstructures were formed on the both surfaces of the Si substrate, and Au microstructures were manufactured by electrolytically plating the insides of the Si microstructures while using the Si microstructures as molds. First, as illustrated in Figs. 2A to 2C, an Si microstructure was formed on the front surface of the Si substrate 10. The formation method thereof may be similar to the method in the first exemplary embodiment as illustrated by Figs. 1A to 1C, and only a difference from the first exemplary embodiment will be described below.

The Si substrate had a diameter of 100 mmϕ, a thickness of 300 µm and a resistivity of 0.02 Ωcm. The formed pattern of the Si microstructure was a line and space (L/S) structure having a pitch p = 6 µm and a width w = 3 µm. The depth of the recessed portion of the Si microstructure was approximately 130 µm. The recessed portion had a width of approximately 3 µm near the front surface and a width of approximately 2.8 µm near the bottom. Therefore, the aspect ratio of the obtained Si groove (recessed portion) was approximately 43. At this point, position alignment marks 80 were formed concurrently as illustrated in Fig. 4A, for the positioning of the Si microstructure on the back surface during the subsequent Si back surface processing.

Next, as illustrated in Fig. 2D, the shape corresponding to the Si structure formed on the front surface of the Si substrate 10 was formed on the back surface of the Si substrate 10 in a substantially mirror-symmetrical manner by applying processing from the back surface. The Si microstructure on the back surface had a nearly similar shape to the shape of the Si microstructure on the front surface, and was positioned with use of the position alignment marks 80 on the front surface of the Si substrate. The Si groove (recessed portion) on the back surface also had a depth of approximately 130 µm and an aspect ratio of approximately 43. The thickness of the layer 16 remaining between the Si microstructures on the front and back surfaces was approximately 40 µm.

Next, as illustrated in Fig. 2E, SiO₂ films having a thickness of approximately 50 nm were formed as second insulating films by heat oxidation on the sidewalls 13 and the bottoms 14 of the Si recessed portions 12 formed by the previous processing. The heat oxidation method enabled the SiO₂ films to be formed concurrently and evenly in the Si microstructures on the front and back surfaces. At this time, the thermal oxidation also progressed even at the portions of the substrate covered with the SiO₂ films, which increases the film thickness of the SiO₂ films.

Next, as illustrated in Fig. 2F, the SiO₂ film 34 formed on the bottom 14 of the Si recessed portion 12 was selectively removed, forming the Si exposed surface 15. This process was performed for each of the Si microstructures on the front and back surfaces. The method for partially removing the SiO₂ film 34 may be similar to the partially removing method in the first example as illustrated in Fig. 1E, and therefore the detailed description thereof will be omitted here. The execution of the above-described processes illustrated in Figs. 2A to 2F led to the formation of the Si mold 40 for plating having the Si microstructures on the both surfaces of the substrate.

Next, as illustrated in Figs. 2G to 2H, the metal microstructures 50 were formed on the both surfaces of the Si substrate by electrolytically plating the insides 12 of the Si structures with Au from the Si exposed surfaces 15 while using the Si molds 40 as molds. The metal electrolytic plating method may be similar to the metal electrolytic plating method in the first example as illustrated in Fig. F, and therefore the detailed description thereof will be omitted here. The heights of the Au microstructures 50 formed in the Si microstructures on the front and back surfaces were controlled by the plating time so as to become approximately 120 µm, respectively. In other words, the aspect ratios of the obtained Au microstructures on the front and back surfaces were approximately 43 respectively, and were approximately 86 in total. A cross-sectional observation with, for example, a SEM revealed that the Au microstructures were dense and had no void. Further, an evaluation with an X-ray microscope confirmed that a grating image with clear contrast could be obtained, and the Au microstructures could absorb X-ray.

As indicated by the present example, the second exemplary embodiment can manufacture high aspect ratio metal structures on the both surfaces of an Si substrate concurrently. This feature can provide not only the effect of a significant reduction in the time required for the manufacturing but also the effect of considerable improvement of the processing accuracy.

In a third example, as illustrated in Figs. 3A to 3J, the Si mold was prepared through a penetrating connection between the microstructures formed on the both surfaces of the Si substrate, and an Au microstructure was manufactured by electrolytically plating the inside of the Si mold. First, as illustrated in Figs. 3A to 3G, the Si substrate 10 was processed so that the Si microstructures were formed and the Si mold 40 was prepared. The processes illustrated in Figs. 3A to 3F may be similar to the processes in the second example as illustrated in Figs. 2A to 2F, and therefore the detailed descriptions thereof will be omitted here.

In the present example, the Si substrate 10 in the state illustrated in Fig. 3F was processed so that the intermediate layer 16 defined between the Si microstructures on the front and back surfaces was removed to penetratingly connect the Si microstructures on the front and back surfaces, as illustrated in Fig. 3G. This process forms the exposed surface 17 on the sidewall of the Si microstructure. This removal of the Si intermediate layer 16 may be performed in a similar manner to the Si etching method in the first example as illustrated in Fig. 1C. After the removal of the Si intermediate layer 16, the substrate was cleaned so that the Si surface could be sufficiently exposed at the exposed surface 17. The processes illustrated in Figs. 3A to 3G resulted in the formation of the Si mold 40 including the penetrating Si microstructure. Here, the depth of the Si groove (recessed portion) was the same as the thickness of the Si substrate, and therefore was 300 µm. In other words, the aspect ratio of the Si groove (recessed portion) was approximately 100.

Next, as illustrated in Figs. 3H to 3J, the Au microstructure 50 was formed by electrolytically plating the inside 12 of the Si structure with Au from the Si exposed surface 17 while using the Si mold 40 including the penetrating Si microstructure. The Au electrolytic plating method may be substantially similar to the electrolytic plating method in the first example and the second example, except for a difference which will be now described. In the present example, the Si microstructure was formed to penetrate and the Si exposed surface 17 was mainly formed on the sidewall of the recessed portion of the Si microstructure. Therefore, in the electrolytic plating of Au, the metal was deposited only on the Si exposed surface 17 in an early stage, as illustrated in Fig. 3H. In other words, the plating solution could pass through the through-hole of the Si microstructure until the deposited Au 50 closed the passage in the Si microstructure as illustrated in Fig. 3I. Due to this feature, the present example had excellent circulation of the plating solution inside the Si microstructure, and therefore was able to provide improved plating efficiency compared to the first and second examples.

Then, as illustrated in Fig. 3J, the Au plating was continued until the thickness of the Au microstructure 50 was increased to approximately 210 µm. In other words, the present example resulted in the formation of an Au microstructure having an aspect ratio of approximately 70. A cross-sectional observation with, for example, a SEM revealed that the Au microstructure was dense and had no void. Further, an evaluation with an X-ray microscope confirmed that a grating image with clear contrast could be obtained, and the Au microstructure could absorb X-ray.

As indicated by the present example, the third exemplary embodiment enables the formation of an Au microstructure having a high aspect ratio with use of the penetrating Si mold. Further, the third exemplary embodiment can provide the following effects in addition to the effects of the first and second examples. First, due to the penetration of the Si microstructure, it is possible to further speed up the formation of a plating core in an early stage of the plating, thereby improving the plating efficiency. Secondly, it is possible to integrate the golden microstructure without the intermediate layer 16 therebetween which exists in the second example. Due to this feature, higher applicability can be expected.

A fourth example will be described with reference to Figs. 5A to 5G. The fourth example used the Si substrate 10 with a diameter of 100 mmϕ, a thickness of 400 µm, and a resistivity of 0.02 Ωcm. Thermally oxidized films with a thickness of approximately 1.0 µm were respectively formed on the front surface and the back surface of the Si substrate 10 as the first insulating films 20 by applying thermal oxidation to the Si substrate 10 at 1050 °C for four hours (Fig. 5A). A chrome film with a thickness of 200 nm was formed on only one surface of the Si substrate 10 by an electron beam evaporation apparatus. A positive type photoresist was applied thereon, and patterning was performed by semiconductor photolithography in such a manner that a square resist pattern 4 µm on a side was two-dimensionally arranged at an 8 µm intervals in an square area 50 mm on a side. After that, the chrome was etched with use of a chrome etching solution, and subsequently, the thermally oxidized film was etched by the reactive etching method with use of CHF₃ to form a Si exposed surface around the resist pattern constituted by the pattern 4 µm on a side two-dimensionally arranged at the 8 µm interval (Fig. 5B).

Next, as illustrated in Fig. 5C, anisotropic deep etching was applied to the Si exposed surface by the inductive coupled plasma-reactive ion etching (ICP-RIE) method. The deep etching was stopped when the deep etching progressed to 70 µm to form a two-dimensional grating composed of Si with a height of 70 µm. Subsequently, the resist and chrome were removed by ultraviolet (UV) ozone ashing and a chrome etching solution. Further, the substrate was cleaned with use of a hydro fluoro ether solution and a mixed solution of sulfuric acid and hydrogen peroxide.

Next, as illustrated in Fig. 5D, a thermally oxidized film with a thickness of approximately 0.15 µm was formed as the second insulating film 30 by applying thermal oxidation at 1050 °C for 15 minutes, on the sidewall 13 of the Si recessed portion formed by the above-mentioned etching. Then, as illustrated in Fig. 5E, the thermally oxidized film formed on the bottom 14 of the Si recessed portion was removed to form the Si exposed surface 15. The partial removal of the thermally oxidized film was performed by the dry etching method with use of CHF₃ plasma. This etching has high anisotropy and progresses nearly vertically relative to a substrate. Therefore, while the thermally oxidized film 34 at the bottom of the Si recessed portion was completely removed, the thermally oxidized film 33 on the sidewall of the Si recessed portion remained so that the Si surface of the sidewall was prevented from being exposed.

Next, a chrome film with a thickness of approximately 7.5 nm and a golden film with a thickness of approximately 55 nm were formed sequentially in this order by an electron beam evaporation apparatus. This processing resulted in the application of a metal film 41 composed of chrome and gold on the Si exposed surface 15 as illustrated in Fig. 5F, which further facilitates generation of a plating core.

Then, the thermally oxidized film formed on the back side of the surface processed by the above-described etching was removed by the dry etching method with use of CHF₃-plasma so that the Si surface was exposed. In the present example, this was used as the mold 40.

Next, as illustrated in Fig. 5G, golden plating was applied by energization through the exposed back side 18 of the Si substrate, as a result of which the metal microstructure 50 was formed. The golden plating was carried out with use non-cyanide gold plating solution (Microfab Au1101: Electroplating Engineers of Japan Ltd.) at 60 °C as the temperature of the plating solution at a current density of 0.2 A/Dm² for 8 hours. This plating resulted in the formation of the metal microstructure 50 made of gold with a thickness of approximately 50 µm. A cross-sectional observation with a SEM revealed that the metal microstructure 50 made of gold was dense, had no void, and had an even height. Further, an evaluation with an X-ray microscope confirmed that a grating image with clear contrast could be obtained, and the metal microstructure 50 made of gold could absorb X-ray.

Next, a fifth example will be described with reference to Figs. 5A to 5G. The fifth example used the Si substrate 10 with a diameter of 100 mmϕ, a thickness of 400 µm, and a resistivity of 0.02 Ωcm. Thermally oxidized films with a thickness of approximately 1.0 µm were respectively formed on the front surface and the back surface of the Si substrate 10 as the first insulating films 20 by applying thermal oxidation to the Si substrate 10 at 1050 °C for four hours (Fig. 5A). A chrome film with a thickness of 200 nm was formed on only one surface of the Si substrate 10 by an electron beam evaporation apparatus. A positive type photoresist was applied thereon, and patterning was performed by semiconductor photolithography in such a manner that a square resist pattern 2 µm on a side was two-dimensionally arranged at 4 µm intervals in a square area 50 mm on a side. After that, the chrome was etched with use of a chrome etching solution, and subsequently, the thermally oxidized film was etched by the reactive etching method with use of CHF₃. As a result, a Si exposed surface was formed around the resist pattern constituted by the pattern 2 µm on a side two-dimensionally arranged at the 4 µm intervals (Fig. 5B).

Next, as illustrated in Fig. 5C, anisotropic deep etching was applied to the exposed Si surface by the ICP-RIE method. The deep etching was stopped when the deep etching progressed to 70 µm. This resulted in the formation of a two-dimensional grating composed of Si with a height of 70 µm. Subsequently, the resist and chrome were removed by UV ozone ashing and a chrome etching solution. Further, the substrate was cleaned with use of a hydro fluoro ether solution and a mixed solution of sulfuric acid and hydrogen peroxide. After the substrate was washed with water, the substrate was immersed in isopropyl alcohol, and then was dried by supercritical drying with use of supercritical carbon dioxide.

Next, as illustrated in Fig. 5D, a thermally oxidized film with a thickness of approximately 0.15 µm was formed as the second insulating film 30 by applying thermal oxidation at 1050 °C for 15 minutes, on the sidewall 13 of the Si recessed portion formed by the above-mentioned etching. Then, as illustrated in Fig. 5E, the thermally oxidized film formed on the bottom 14 of the Si recessed portion was removed, as a result of which the Si exposed surface 15 was formed. The partial removal of the thermally oxidized film was performed by the dry etching method with use of CHF₃ plasma. This etching has high anisotropy and progresses nearly vertically relative to a substrate. Therefore, while the thermally oxidized film 34 at the bottom of the Si recessed portion was completely removed, the thermally oxidized film 33 on the sidewall of the Si recessed portion remained so that the Si surface of the sidewall was prevented from being exposed.

Next, a chrome film with a thickness of approximately 7.5 nm and a copper film with a thickness of approximately 50 nm were formed sequentially in this order by an electron beam evaporation apparatus. This processing applies a metal film 41 composed of chrome and copper on the Si exposed surface 15 as illustrated in Fig. 5F. Since copper has a greater ionization tendency than gold, the copper surface on the bottom 14 of the Si recessed portion is displaced by gold when being immersed in a gold plating solution, which facilitates generation of a gold plating nucleus. Further, the copper slightly attached to the side wall 13 of the Si recessed portion at the time of electron beam evaporation is dissolved and removed. Therefore, development of the plating is facilitated on the bottom 14 of the Si recessed portion.

Then, the thermally oxidized film formed on the back side of the surface processed by the above-described etching was removed by the dry etching method with use of CHF₃-plasma so that the Si surface was exposed. In the present example, this was used as the mold 40.

Next, as illustrated in Fig. 5G, golden plating was applied by energization through the exposed back side 18 of the Si substrate, as a result of which the metal microstructure 50 was formed. The golden plating was carried out with use of a non-cyanide gold plating solution (Microfab Au1101: Electroplating Engineers of Japan Ltd.) at 60 °C as the temperature of the plating solution at a current density of 0.2 A/dm² for 8 hours. This plating forms the metal microstructure 50 made of gold with a thickness of approximately 50 µm. A cross-sectional observation with a SEM revealed that the metal microstructure 50 made of gold was dense, had no void, and had an even height, and further, the surface of the metal microstructure 50 in the Si recessed portion 12 was flat. Further, an evaluation with an X-ray microscope confirmed that a grating image with clear contrast could be obtained, and the metal microstructure 50 made of gold could absorb X-ray.

The microstructure manufacturing method according to the present example enables easy manufacturing of a metal microstructure having a high aspect ratio with a high degree of precision, and the resulting metal microstructure can be utilized for, for example, an X-ray absorption grating, an X-ray beam splitter, a photonic crystal, a metamaterial, and a metal mesh for a transmission electronic microscope.

In the following, an imaging apparatus utilizing the X-ray Talbot interference method will be described with reference to Fig. 6. Fig. 6 illustrates a configuration of an imaging apparatus using the microstructure manufactured in the above-described exemplary embodiments or examples as an X-ray absorption grating.

The imaging apparatus according to the present exemplary embodiments includes an X-ray source 100 for emitting spatially coherent X-ray, a diffraction grating 200 for periodically modulating the phase of the X-ray, an absorption grating 300 in which an X-ray absorption portion (shield portion) and a transmission portion are arranged, and a detector 400 for detecting the X-ray. The absorption grating 300 is the microstructure manufactured by the above-described exemplary embodiments or examples.

When a subject 500 is positioned between the X-ray source 100 and the diffraction grating 200, information about X-ray phase shift due to the subject 500 is detected as moire by the detector. In other words, this imaging apparatus captures an image of the subj ect 500 by imaging moire which holds phase information of the subject 500. Execution of phase retrieval processing such as Fourier transform based on this detection result enables a phase image of the subject to be obtained.

Since the imaging apparatus according to the present exemplary embodiments uses a less defective absorption grating, it can capture a phase image of a subject more accurately.

## Claims

1. A microstructure manufacturing method comprising:
forming a first insulating film on an Si substrate;
exposing an Si surface by removing a part of the first insulating film;
forming a recessed portion by etching the Si substrate from the exposed Si surface;
forming a second insulating film the thickness of which is within a range of 5 nm to 5000 nm on a sidewall and a bottom of the recessed portion;
forming an Si exposed surface by removing at least a part of the second insulating film formed on the bottom of the recessed portion; and
filling the recessed portion with a metal from the Si exposed surface by electrolytic plating.

2. The microstructure manufacturing method according to claim 1, comprising:
forming the first insulating film on each of a front surface and a back surface of the Si substrate in the first insulating film formation;
exposing the Si surface of the Si substrate by removing a part of the first insulating film on the front surface of the Si substrate in the Si surface exposure, and then forming the Si recessed portion on the front surface of the Si substrate by etching the Si substrate from the exposed Si surface while using the first insulating film on the front surface of the Si substrate as a mask;
exposing the Si surface of the Si substrate by removing a part of the first insulating film on the back surface of the Si substrate, and then forming the Si recessed portion on the back surface of the Si substrate by etching the Si substrate from the exposed Si surface while using the first insulating film on the back surface of the Si substrate as a mask in the recessed portion formation;
forming the second insulating film over the sidewall and the bottom of the Si recessed portion of each of the front surface and the back surface of the Si substrate in the second insulating film formation;
forming the Si exposed surface by removing at least a part of the second insulating film formed over the bottom of the Si recessed portion of each of the front surface and the back surface of the Si substrate in the Si exposed surface formation; and
forming the metal microstructure by filling the Si recessed portion with the metal by electrolytic plating from the Si exposed surface on each of the front surface and the back surface of the Si substrate in the metal filling.

3. The microstructure manufacturing method according to claim 2, wherein the Si substrate is etched from the exposed Si surface with use of the first insulating film over each of the front surface and the back surface of the Si substrate as a mask, and the Si recessed portions on the front surface and the back surface of the Si substrate are formed either in a manner that the Si recessed portions penetrate or in a manner that the Si recessed portions do not penetrate.

4. The microstructure manufacturing method according to any one of claims 1 to 3, wherein the Si substrate has a resistivity of 10 Ωcm or less.

5. The microstructure manufacturing method according to any one of claims 1 to 4, further comprising:
applying a metal film on the exposed Si surface of the bottom,
wherein the recessed portion is filled with a metal from the metal film by electrolytic plating.

6. The microstructure manufacturing method according to claim 5, the metal film includes a metal having a greater ionization tendency than the ionization tendency of the metal.

7. The microstructure manufacturing method according to any one of claims 1 to 6,
wherein the electrolytic plating is carried out with use of a non-cyanide plating solution, and
wherein a material of the second insulating film is SiO₂.

8. The microstructure manufacturing method according to any one of claims 1 to 7, wherein the first insulating film is thicker than the second insulating film formed on the bottom on the recessed portion.

9. An X-ray absorption grating comprising:
an Si substrate including a plurality of recessed portions or holes; and
a metal filled in each of the plurality of recessed portions or holes via an insulating film the thickness of which is within a range of 5 nm to 5000 nm,
wherein the insulating film is not formed on at least a part of a bottom of the recessed portion.

10. The X-ray absorption grating according to claim 9, wherein the metal is in contact with an Si surface of the Si substrate at least on the part.

11. The X-ray absorption grating according to claim 9, wherein the Si substrate includes the plurality of recessed portions, and
wherein a metal film is disposed between an Si surface of the Si substrate and the metal at least on the part.

12. The X-ray absorption grating according to claim 11, the metal film includes a metal having a greater ionization tendency than the ionization tendency of the metal which is filled in the recessed portion.

13. The X-ray absorption grating according to any one of claims 9 to 12, the metal which is filled in each of the plurality of recessed portions or holes has an aspect ratio of 0.1 to 150.

14. An imaging apparatus for capturing an image of a subject, comprising:
an X-ray source;
a diffraction grating for diffracting X-ray emitted from the X-ray source;
an absorption grating for absorbing a part of the X-ray diffracted by the diffraction grating, the absorption grating being the X-ray absorption grating according to any one of claims 9 to 13; and
a detector for detecting the X-ray which has passed through the absorption grating.

## Patentansprüche

1. Mikrostrukturherstellungsverfahren, das Folgendes umfasst:
Ausbilden einer ersten Isolierschicht auf einem Si-Substrat;
Freilegen einer Si-Oberfläche durch Entfernen eines Teils der ersten Isolierschicht;
Ausbilden eines Vertiefungsabschnitts durch Ätzen des Si-Substrats von der freiliegenden Si-Oberfläche aus;
Ausbilden einer zweiten Isolierschicht, deren Dicke auf einer Seitenwand und einem Boden des Vertiefungsabschnitts in einem Bereich von 5 nm bis 5000 nm liegt;
Ausbilden einer Si-Freilegeoberfläche durch Entfernen zumindest eines Teils der zweiten Isolierschicht, die auf dem Boden des Vertiefungsabschnitts ausgebildet ist; und
Füllen des Vertiefungsabschnitts mit einem Metall von der Si-Freilegeoberfläche aus durch elektrolytisches Beschichten.

2. Mikrostrukturherstellungsverfahren nach Anspruch 1, das Folgendes umfasst:
bei der ersten Isolierschichtausbildung Ausbilden der ersten Isolierschicht auf jeweils einer Vorderseite und einer Rückseite des Si-Substrats;
bei der Si-Oberflächenfreilegung Freilegen der Si-Oberfläche des Si-Substrats durch Entfernen eines Teils der ersten Isolierschicht auf der Vorderseite des Si-Substrats, und dann Ausbilden des Si-Vertiefungsabschnitts auf der Vorderseite des Si-Substrats durch Ätzen des Si-Substrats von der freiliegenden Si-Oberfläche aus, während die erste Isolierschicht auf der Vorderseite des Si-Substrats als eine Maske verwendet wird;
Freilegen der Si-Oberfläche des Si-Substrats durch Entfernen eines Teils der ersten Isolierschicht auf der Rückseite des Si-Substrats, und dann bei der Vertiefungsabschnittausbildung Ausbilden des Si-Vertiefungsabschnitts auf der Rückseite des Si-Substrats durch Ätzen des Si-Substrats von der freiliegenden Si-Oberfläche aus, während die erste Isolierschicht auf der Rückseite des Si-Substrats als eine Maske verwendet wird;
bei der zweiten Isolierschichtausbildung Ausbilden der zweiten Isolierschicht über der Seitenwand und dem Boden des Si-Vertiefungsabschnitts von jeweils der Vorderseite und der Rückseite des Si-Substrats;
bei der Si-Freilegeoberflächenausbildung Ausbilden der Si-Freilegeoberfläche durch Entfernen zumindest eines Teils der zweiten Isolierschicht, die über dem Boden des Si-Vertiefungsabschnitts von jeweils der Vorderseite und der Rückseite des Si-Substrats ausgebildet ist; und
Ausbilden der Metallmikrostruktur, indem beim Metallfüllen der Si-Vertiefungsabschnitts von der Si-Freilegeoberfläche auf jeweils der Vorderseite und der Rückseite des Si-Substrats aus durch elektrolytisches Beschichten mit dem Metall gefüllt wird.

3. Mikrostrukturherstellungsverfahren nach Anspruch 2, wobei das Si-Substrat von der freiliegenden Si-Oberfläche aus mit Hilfe der ersten Isolierschicht über jeweils der Vorderseite und der Rückseite des Si-Substrats als einer Maske geätzt wird und die Si-Vertiefungsabschnitte auf der Vorderseite und der Rückseite des Si-Substrats entweder auf eine Weise, dass die Si-Vertiefungsabschnitte durchdringen, oder auf eine Weise, dass die Si-Vertiefungsabschnitte nicht durchdringen, ausgebildet werden.

4. Mikrostrukturherstellungsverfahren nach einem der Ansprüche 1 bis 3, wobei das Si-Substrat einen Widerstand von 10 Ωcm oder weniger hat.

5. Mikrostrukturherstellungsverfahren nach einem der Ansprüche 1 bis 4, das außerdem Folgendes umfasst:
Aufbringen einer Metallschicht auf der freiliegenden Si-Oberfläche des Bodens,
wobei der Vertiefungsabschnitt von der Metallschicht aus durch elektrolytisches Beschichten mit einem Metall gefüllt wird.

6. Mikrostrukturherstellungsverfahren nach Anspruch 5, wobei die Metallschicht ein Metall enthält, das eine größere Ionisationstendenz als die Ionisationstendenz des Metalls hat.

7. Mikrostrukturherstellungsverfahren nach einem der Ansprüche 1 bis 6,
wobei das elektrolytische Beschichten mit Hilfe einer Nicht-Cyanid-Beschichtungslösung erfolgt und
wobei ein Material der zweiten Isolierschicht SiO₂ ist.

8. Mikrostrukturherstellungsverfahren nach einem der Ansprüche 1 bis 7, wobei die erste Isolierschicht dicker als die zweite Isolierschicht, die auf dem Vertiefungsabschnitt auf dem Boden ausgebildet ist, ist.

9. Röntgenstrahl-Absorptionsgitter mit:
einem Si-Substrat, das eine Vielzahl von Vertiefungsabschnitten oder Löchern aufweist; und
einem Metall, das über eine Isolierschicht, deren Dicke in einem Bereich von 5 nm bis 5000 nm liegt, in jeden der Vielzahl von Vertiefungsabschnitten oder jedes der Vielzahl von Löchern eingefüllt ist,
wobei die Isolierschicht nicht auf zumindest einem Teil eines Bodens des Vertiefungsabschnitts ausgebildet ist.

10. Röntgenstrahl-Absorptionsgitter nach Anspruch 9, wobei sich das Metall zumindest auf dem Teil mit einer Si-Oberfläche des Si-Substrats in Kontakt befindet.

11. Röntgenstrahl-Absorptionsgitter nach Anspruch 9, wobei das Si-Substrat die Vielzahl von Vertiefungsabschnitten enthält und
wobei zumindest auf dem Teil zwischen einer Si-Oberfläche des Si-Substrats und dem Metall eine Metallschicht angeordnet ist.

12. Röntgenstrahl-Absorptionsgitter nach Anspruch 11, wobei die Metallschicht ein Metall enthält, das eine größere Ionisationstendenz als die Ionisationstendenz des Metalls, das in dem Vertiefungsabschnitt eingefüllt ist, hat.

13. Röntgenstrahl-Absorptionsgitter nach einem der Ansprüche 9 bis 12, wobei das Metall, das in jeden der Vielzahl von Vertiefungsabschnitten oder jedes der Vielzahl von Löchern eingefüllt ist, ein Längenverhältnis von 0,1 bis 150 hat.

14. Bilderzeugungsgerät zum Erfassen eines Bilds eines Gegenstands, mit:
einer Röntgenstrahlquelle;
einem Beugungsgitter zum Beugen eines von der Röntgenstrahlquelle abgegebenen Röntgenstrahls;
einem Absorptionsgitter zum Absorbieren eines Teils des durch das Beugungsgitter gebeugten Röntgenstahls, wobei das Absorptionsgitter das Röntgenstrahl-Absorptionsgitter gemäß einem der Ansprüche 9 bis 13 ist; und
einem Detektor zum Erfassen des Röntgenstrahls, der durch das Absorptionsgitter gegangen ist.

## Revendications

1. Procédé de fabrication de microstructure comprenant le fait :
de former un premier film isolant sur un substrat de Si ;
d'exposer une surface de Si par retrait d'une partie du premier film isolant ;
de former une partie en évidement par gravure du substrat de Si à partir de la surface de Si exposée ;
de former un deuxième film isolant dont l'épaisseur se trouve dans une plage allant de 5 nm à 5000 nm sur une paroi latérale et le fond de la partie en évidement ;
de former une surface exposée de Si par retrait d'au moins une partie du deuxième film isolant formé sur le fond de la partie en évidement ; et
de remplir la partie en évidement d'un métal à partir de la surface exposée de Si par un dépôt électrolytique.

2. Procédé de fabrication de microstructure selon la revendication 1, comprenant le fait :
de former le premier film isolant sur chacune d'une surface avant et d'une surface arrière du substrat de Si lors de la formation du premier film isolant ;
d'exposer la surface de Si du substrat de Si par retrait d'une partie du premier film isolant sur la surface avant du substrat de Si lors de l'exposition de la surface de Si, et de former ensuite la partie en évidement de Si sur la surface avant du substrat de Si par gravure du substrat de Si à partir de la surface de Si exposée tout en utilisant le premier film isolant sur la surface avant du substrat de Si en tant que masque ;
d'exposer la surface de Si du substrat de Si par retrait d'une partie du premier film isolant sur la surface arrière du substrat de Si, et de former ensuite la partie en évidement de Si sur la surface arrière du substrat de Si par gravure du substrat de Si à partir de la surface de Si exposée tout en utilisant le premier film isolant sur la surface arrière du substrat de Si en tant que masque lors de la formation de la partie en évidement ;
de former le deuxième film isolant sur la paroi latérale et le fond de la partie en évidement de Si de chacune de la surface avant et de la surface arrière du substrat de Si lors de la formation du deuxième film isolant ;
de former la surface exposée de Si par retrait d'au moins une partie du deuxième film isolant formé sur le fond de la partie en évidement de Si de chacune de la surface avant et de la surface arrière du substrat de Si lors de la formation de la surface exposée de Si ; et
de former la microstructure métallique en remplissant la partie en évidement de Si du métal par un dépôt électrolytique à partir de la surface exposée de Si sur chacune de la surface avant et de la surface arrière du substrat de Si lors du remplissage métallique.

3. Procédé de fabrication de microstructure selon la revendication 2, dans lequel le substrat de Si est gravé à partir de la surface de Si exposée en utilisant le premier film isolant sur chacune de la surface avant et de la surface arrière du substrat de Si en tant que masque, et les parties en évidement de Si sur la surface avant et la surface arrière du substrat de Si sont formées soit de manière à ce que les parties en évidement de Si pénètrent ou de manière à ce que les parties en évidement de Si ne pénètrent pas.

4. Procédé de fabrication de microstructure selon l'une quelconque des revendications 1 à 3, dans lequel le substrat de Si a une résistivité inférieure ou égale à 10 Ωcm.

5. Procédé de fabrication de microstructure selon l'une quelconque des revendications 1 à 4, comprenant en outre le fait :
d'appliquer un film métallique sur la surface de Si exposée du fond,
dans lequel la partie en évidement est remplie d'un métal à partir du film métallique par un dépôt électrolytique.

6. Procédé de fabrication de microstructure selon la revendication 5, le film métallique comporte un métal ayant une tendance à l'ionisation supérieure à la tendance à l'ionisation du métal.

7. Procédé de fabrication de microstructure selon l'une quelconque des revendications 1 à 6,
dans lequel le dépôt électrolytique est effectué en utilisant une solution de dépôt sans-cyanure, et
dans lequel un matériau du deuxième film isolant est du SiO₂.

8. Procédé de fabrication de microstructure selon l'une quelconque des revendications 1 à 7, dans lequel le premier film isolant est plus épais que le deuxième film isolant formé sur le fond de la partie en évidement.

9. Réseau d'absorption des rayons X comprenant :
un substrat de Si comportant une pluralité de trous ou de parties en évidement ; et
un métal introduit dans chacun(e) de la pluralité de trous ou de parties en évidement par l'intermédiaire d'un film isolant dont l'épaisseur se trouve dans une plage allant de 5 nm à 5000 nm,
dans lequel le film isolant n'est pas formé sur au moins une partie du fond de la partie en évidement.

10. Réseau d'absorption des rayons X selon la revendication 9, dans lequel le métal est en contact avec une surface de Si du substrat de Si au moins sur la partie.

11. Réseau d'absorption des rayons X selon la revendication 9, dans lequel le substrat de Si comporte la pluralité de parties en évidement, et
dans lequel un film métallique est disposé entre une surface de Si du substrat de Si et le métal au moins sur la partie.

12. Réseau d'absorption des rayons X selon la revendication 11, le film métallique comporte un métal ayant une tendance à l'ionisation supérieure à la tendance à l'ionisation du métal qui est introduit dans la partie en évidement.

13. Réseau d'absorption des rayons X selon l'une quelconque des revendications 9 à 12, le métal qui est introduit dans chacun (e) de la pluralité de trous ou de parties en évidement a un rapport d'aspect compris entre 0,1 et 150.

14. Appareil d'imagerie pour capturer une image d'un sujet, comprenant :
une source de rayons X ;
un réseau de diffraction pour diffracter un rayon X émis à partir de la source de rayons X ;
un réseau d'absorption pour absorber une partie du rayon X diffracté par le réseau de diffraction, le réseau d'absorption étant le réseau d'absorption des rayons X selon l'une quelconque des revendications 9 à 13 ; et
un détecteur pour détecter le rayon X qui a traversé le réseau d'absorption.
